

April 28, 1970

J. E. MATSON

3,508,428

CONNECTOR ELEMENT FOR RIGID ELECTRICAL CONDUITS AND  
METHOD OF MAKING THE SAME

Filed Dec. 5, 1968



Fig. 1.



Fig. 2.



Fig. 5.



Fig. 3.



Fig. 4.



Fig. 6.

Inventor  
James Edward Matson

By Mann, Brown  
and McWilliams,  
Atlys.

1

3,508,428  
**CONNECTOR ELEMENT FOR RIGID ELECTRICAL CONDUITS AND METHOD OF MAKING THE SAME**

James Edward Matson, Galva, Ill., assignor to All-Steel Equipment Inc., a corporation of Illinois  
Continuation-in-part of application Ser. No. 652,189, July 10, 1967. This application Dec. 5, 1968, Ser. No. 786,540

Int. Cl. B21d 11/04

U.S. CL. 72—327

4 Claims

## ABSTRACT OF THE DISCLOSURE

Hollow connector elements for rigid electrical conduits are formed with internal shoulders by displacing metal inwardly from one end of the element by means of a special swaging or forging tool without the use of an outer supporting die and without substantially changing the outer size or shape of the element.

This application is a continuation-in-part of application Ser. No. 652,189, now abandoned, entitled Connector Element for Rigid Electrical Conduits and Method of Making the Same, filed July 10, 1967.

## SUMMARY OF THE INVENTION

In making connector elements for rigid electrical conduits it has been the practice to neck a portion of larger diameter hollow tubular stock to a small diameter and then thread the necked portion. This method is relatively expensive.

In accordance with the present invention, metal is squeezed inwardly or swaged from one end portion of the connector element thereby displacing this metal in the form of an annular shoulder having a smooth flat face on the side from which metal was displaced. The resulting connector element will have a wall portion on the side of the shoulder from which the metal was displaced which is thinner than the remaining wall portion of the connector. The inner surface of the thinner wall portion is smooth as a result of the swaging operation. The shoulder will extend radially inward beyond the inner surface of the thicker portion of the connector element. The operation is performed in one step with a special swaging tool or punch and without a retaining die, thus avoiding the problem of freeing the piece from the die and enabling the operation to be performed rapidly. The resulting shoulder is a substantially perfect annular ring with a smooth top surface and requires no machining or trimming operation. The operation does not substantially change the size or shape of the outer wall of the element. A threaded hole is then formed through the side wall of the connector element to accommodate a set screw and a separate threaded element is fastened to the connector element just described by beading the thinner wall end of the connector element around an outwardly extending flange on one end of the threaded member, which flange rests on the smooth face of the shoulder.

2

## BRIEF DESCRIPTION OF THE DRAWINGS

FIGURE 1 is a diagrammatic, vertical view of a connector element prior to having a shoulder formed therein in accordance with the invention.

FIGURE 2 is a cross-section of the element shown in FIGURE 1 taken along the line 2—2.

FIGURE 3 is a vertical cross-sectional view of a connector element showing the manner in which the internal shoulder is formed.

FIGURE 4 is a vertical cross-sectional view of the connector element shown in FIGURE 3 after the mandrel and swaging tool have been removed.

FIGURE 5 is a vertical cross-sectional view showing the connector element formed in accordance with the invention with a threaded element in place ready to be fastened.

FIGURE 6 is a vertical cross-sectional view showing the finished connector after the end of the connector element made in accordance with the invention has been beaded over the flanged end of the threaded element.

## DETAILED DESCRIPTION OF THE INVENTION

One of the objects of the invention is to provide a novel connector element for rigid electrical conduits.

Still another object of the invention is to provide a novel method for forming a connector element having an internal shoulder.

A further object of the invention is to provide apparatus for forming an internal shoulder in a hollow element in a high speed operation.

Other objects of the invention will become apparent from the following description and the accompanying drawing.

In the drawing, the numeral 1 indicates a hollow, cylindrical metal element which may be made of steel, brass, aluminum, or other metal which can be deformed but preferably C1010 or C1015 cold drawn steel tubing. In order to prepare the novel connector element of this invention the hollow cylindrical piece 1 is centered below stamping tool 2 by means of supporting plate 3 and mandrel 4 fastened to the supported plate by bolt 5. A cylindrical swaging or forging element 7 having an outside diameter intermediate between the diameter of the outer wall 9 and the inner wall 11 of the cylindrical piece 1 is mounted on the lower end of tool 2 by retainer 12 which in turn is fastened to tool 2 by means of bolt 13. As shown in FIGURE 3, retainer 12 is formed with shoulder 12' which abuts the end of element 7 and is tapered upwardly from its leading surface and outwardly to a maximum diameter equal to that of the diameter of the opening defined by shoulder 14 and determines the width of the shoulder. As shown in the drawing the exposed wall of the retainer element is frusto-conical. Although the retainer is shown with a slightly sloping wall it may be formed with a wall substantially parallel to the wall of element 1. The retainer 12 is of sufficient depth or thickness to confine the metal, forged from the inner wall of element 1, between the element wall and the retainer during the entire swaging or forging operation. By providing contiguous wall elements spaced apart a distance equal to the width of the desired shoulder between which the shoulder forms and is squeezed or com-

pressed, a finished shoulder is formed in a single stroke or operation. As is evident from FIGURE 3, the shoulder is not squeezed against the bottom mandrel 4 and as a result the lower surface of the shoulder is curved. By forcing tool 2 against the top end 15 of piece 1, metal adjacent the inner wall of the element is displaced and forced in the direction of mandrel 4. The diameter of the swaging tool 7 is preferably closer to that of the inner diameter of the element 1 than the outer diameter thereof so that after the metal is displaced from the wall the thickness of the portion of the wall 16 above the shoulder 14 will be more than half the thickness of the portion of the wall 17 below the shoulder. The swaging operation is discontinued when the shoulder 14 has been formed at the desired locus. As an example, a connector element made of C1010 or C1015 cold drawn, butt welded steel, having a length of  $1\frac{1}{16}$  inches, an outer diameter of 1.125 inches and an inner diameter between .865 and .875 inch so that the wall thickness is between 0.13 and 0.125 inch, is swaged in accordance with my invention to form a shoulder at a depth of 0.156 inch from the end to which the swaging element is applied, with the shoulder extending radially inwardly a distance between 0.1675 and 0.1685 inch from the inner wall from which the shoulder metal is displaced. The resulting connector element wall above the shoulder will have its thickness reduced between 0.046 and 0.040 inch. The thickness of this portion of the wall was reduced by about  $\frac{1}{3}$ .

As another example, an element made of C1010 or C1015 cold drawn, butt welded steel tubing having a length of  $1\frac{5}{8}$  inches, outside wall diameter of 1.312 inches and inside wall diameter between 1.075 and 1.085 inches, was swaged to form a shoulder at a distance of 0.133 inch from one end. The diameter of the opening defined by the resulting shoulder was about 0.906 inch and the thickness of the wall from which metal was displaced was about 0.058 inch. The thickness of the latter wall was reduced about 48%.

As another example, C1010 or C1015 cold drawn, butt welded steel tubing having a length of  $1\frac{3}{16}$  inches, outside wall diameter of 1.625 inches and inside wall diameter of 1.340 to 1.350 inches, was swaged to form a shoulder at a distance of 0.172 inch from one end. The diameter of the opening defined by the resulting shoulder was about 1.188 inches and the thickness of the wall from which metal was displaced was about 0.087 inch. The thickness of the latter wall was reduced about 37.5%.

The thickness of the wall from which metal is displaced should not be less than about 0.1 to 0.15 inch since undesirable distortion of the tubular element may occur during the swaging operation if the wall is too thin. On the other hand, the amount of metal swaged from the interior of the tubular piece must be sufficient to form a solid mass of shoulder integral with the interior surface of the piece. We have found that by limiting the thickness swaged or displaced from the wall to about 0.04 to 0.06 inch excellent results are obtained with high speed production. It should be understood that tubular stock having a wall thickness greater than that of the aforesaid examples may be used provided the thickness of the metal swaged to form the shoulder is of the order of .04 to .06 inch.

The connector element after the shoulder has been formed by the aforesaid swaging operation is shown in FIGURE 4. It will be noted that the upper face 19 of the shoulder 14 is smooth and flat, whereas the under face 21 has a curved surface gradually increasing in thickness from the inner circular periphery to the line of juncture with the wall portion 17. The inner wall 18, formed by removing metal to form the shoulder, is also smooth, as if it had been machined.

By carefully controlling the thickness of metal displaced from the inner wall of the element, the swaging

operation can be performed without the necessity of using a supporting or retaining die fitting closely around the outer wall of the element which would ordinarily be required to prevent distortion of the element during the swaging operation. When using a retaining die distortion of the element during the swaging operation results in binding between the die and element and the attendant problem of freeing the two from each other. By reason of the fact that a retaining die is not used the swaging operation can be performed rapidly since the problem of freeing the element from the retaining die is avoided.

The connector element, after the shoulder has been formed is designated generally by the numeral 23. In making a finished connector, the element 23 has a threaded hole 25 (FIGURES 5 and 6) formed in the wall below the shoulder 14 in order to enable a set screw to be threaded therein and screwed against an electrical conduit (not shown) which is inserted into the element 23. A threaded hollow element 27 having an outwardly extending flange 29 the circumference of which is slightly less than that of the inner wall 22 is placed in the element 23 with the flange resting on the shoulder 14. The upper end 15 of the element 23 is then beaded over the flange 29 as shown at 31 (FIGURE 6), thereby fastening the element 27 securely to the element 23 and forming a finished connector.

It will be apparent how the finished connector shown in FIGURE 6 is utilized. The threaded element 23 is inserted in a hole in an electrical box until the beaded end 31 abuts against the outside of the box and a lock nut is then threaded on the element 27 on the inside of the box to hold the connector securely in the box.

Connector elements in accordance with the invention are produced on automatic, intermittent high speed stamping presses. Speeds of 35 to 40 units per minute can be made with each swaging tool. The speed of production of connectors made in accordance with my invention has been increased ten-fold over the speed of production by methods heretofore used, with a resulting significant reduction in cost. This has been made possible by eliminating the use of an outside die thereby avoiding the difficulty in removing the piece from the die after the swaging operation. When an outside die is used, the connector element binds to the die due to the slight expansion in circumference of the element in the area of the swaging or forging operation.

Although specific examples have been given it will be understood that connectors of different sizes can be made in accordance with the invention. The wall thickness of the connector element should be sufficient to swage metal therefrom to form the shoulder and leave sufficient wall length and thickness to form a bead.

Although the invention has been described as applied to the formation of shoulders in steel connector elements, it is applicable to formation of shoulders in other types of hollow pieces made of sufficiently ductile material to be drawn or forged.

I claim:

1. The method of forming a shoulder interiorly of a hollow, open-ended element having a wall thickness not less than about 0.1 inch and made of material sufficiently ductile to be forged, comprising centering and supporting said element concentrically below a swaging tool by means of a plate and mandrel at the lower end of said element, the outer periphery of which tool corresponds to that of the periphery of the inner wall of said element but has a diameter approximately .08 to .12 inch greater than that of said inner wall, forcing said tool downwardly against the upper end of said element with sufficient force to displace metal from the interior of said element while the outer wall of the upper end of said element is unconfined by a supporting die, providing a confining wall adjacent the bottom of said tool, said confining wall being concentric with the outer periphery of the inner wall of said element.

tric with the inner wall of said element and spaced therefrom a distance equal to the width of the desired shoulder thereby to form an annular space between the inner wall and confining wall, continuing to displace metal from said element into said annular space until the shoulder has attained the desired width and withdrawing the tool from the element.

2. The method in accordance with claim 1 in which the element is made of steel and has a wall thickness of approximately 0.1 to 0.15 inch. 10

3. The method in accordance with claim 2 in which the shoulder is formed without supporting the surface thereof opposite that contacted by the swaging tool.

4. Method in accordance with claim 1 in which the 15 confining wall adjacent the bottom of said tool is frustoconical in shape with the wall sloping outwardly from its leading end.

## References Cited

## UNITED STATES PATENTS

|           |        |          |       |        |
|-----------|--------|----------|-------|--------|
| 1,412,196 | 4/1922 | Rabold   | ----- | 72—370 |
| 2,583,270 | 1/1952 | Lynall   | ----- | 72—358 |
| 2,679,681 | 6/1954 | Resler   | ----- | 72—370 |
| 2,800,247 | 7/1957 | Appleton | ----- | 29—511 |
| 382,924   | 5/1888 | Wilcox   | ----- | 72—464 |
| 3,436,803 | 4/1969 | Sarnoff  | ----- | 29—511 |

## FOREIGN PATENTS

|         |        |         |
|---------|--------|---------|
| 583,088 | 6/1924 | France. |
| 594,670 | 3/1925 | France. |

CHARLES W. LANHAM, Primary Examiner

E. M. COMBS, Assistant Examiner

U.S. CL. X.R.

72—359, 370, 377